

Feb. 6, 1940.

L. E. FLORY

2,189,322

PHOTOELECTRIC CATHODE

Filed Jan. 19, 1937



Fig. 1

Fig. 3.



Fig. 2.



Inventor  
Leslie E. Flory  
J. J. Jaff  
By  
Attorney

## UNITED STATES PATENT OFFICE

2,189,322

## PHOTOELECTRIC CATHODE

Leslie E. Flory, Oaklyn, N. J., assignor to Radio Corporation of America, a corporation of Delaware

Application January 19, 1937, Serial No. 121,259

8 Claims. (Cl. 250—165)

My invention relates to photoelectric cathodes and particularly to cathodes of the type which are transparent or semi-transparent.

In various electronic tubes, cathodes of the above-mentioned type are desirable. For example, in the image amplifier described and claimed in application Serial No. 55,957, filed December 24, 1935, in the name of George A. Morton and assigned to the Radio Corporation of America, the cathode should be transparent whereby an optical image projected on one side of the cathode will release electrons on the opposite side thereof.

An object of my invention is to provide an improved cathode of the above-mentioned type.

15 A further object of my invention is to provide an improved method of making a cathode of the above-mentioned type.

In practicing my invention, I form a transparent layer of silver oxide on a transparent supporting surface, then sensitize the silver oxide layer by caesium or the like, and finally form a transparent layer of silver on the sensitized surface. The final layer of silver gives the cathode the necessary conductivity (the base layer of silver oxide being an insulator) and also increases the photo-electric sensitivity.

The invention will be better understood from the following description taken in connection with the accompanying drawing in which:

30 Fig. 1 is a view of an image amplifier tube embodying my invention.

Fig. 2 is a view taken on the line 2—2 of Fig. 1, and

35 Fig. 3 is a view in cross-section on an enlarged scale of the cathode shown in Fig. 1.

In Fig. 1, I have shown my invention applied to an image amplifier tube of the type described and claimed in the above-mentioned Morton application. This tube comprises a highly evacuated glass envelope 1 having a semi-transparent fluorescent screen 2 on one end thereof. A transparent photoelectric cathode 3 hereinafter described is located at the other end of the glass envelope.

45 Located coaxially along the tube between the cathode 3 and the screen 2 are a plurality of focusing rings 4, 6, 7, 8 and 9, and an anode 11 which may be in the form of a foraminous cylinder. A suitable voltage source such as a battery 12 maintains the anode 11 highly positive with respect to the cathode 3.

50 The focusing rings 4, 6, 7, 8 and 9 are maintained at successively higher positive potentials by connections to points on a potentiometer 13

comprising a plurality of resistors connected in series. One end of potentiometer 13 is connected to the cathode 3 through a metallized edge 5 and to the negative end of battery 12, while the other end of the potentiometer is connected through a variable tap to a point on a potentiometer 14 shunted across battery 12.

5 As described in the above-identified Morton application, flanges or discs 16 and 17 are supported from and electrically connected to the 10 ring 9 and the anode 11, respectively, for the purpose of producing the desired magnification of an image projected upon cathode 3 and appearing upon screen 2.

In accordance with one feature of my invention, 15 I attach an inner shielding ring 18 to the disc 16 and support a circular filament 19 between the shielding ring 18 and the focusing ring 9 as shown more clearly in Fig. 2. Silver beads 21 are located at intervals on the filament 19 whereby silver 20 may be vaporized by heating the filament. The shielding ring 18 tends to keep the silver off the rings 4, 6, 7 and 8 and the resistors 13 and to direct the silver vapor toward the cathode 3 where it forms a silver layer thereon during the process 25 of making the cathode.

The specific structure of the cathode 3 and the method of making it will now be described. Referring to Fig. 3, the cathode comprises a transparent supporting member 26 which preferably is 30 of glass or mica. In the particular tube illustrated it is a circular convex member similar to a watch crystal. The photoelectric surface on the member 26 consists of three more or less distinct layers, the first one being a transparent layer 27 of silver oxide, the next one being a transparent layer 28 of photoelectric material such as caesium oxide or the like, and the outside layer 29 being a transparent layer of silver. This description of the several layers on the glass surface may not be strictly correct as it is difficult to determine the exact nature of such structure, but it is believed to be substantially correct.

35 The nature of the cathode 2 will be better understood by a description of the way in which it is produced. The photoelectric surface is formed on the supporting member 26 after the tube shown in Fig. 1 has been completely assembled. First, the assembled tube is baked and pumped to a high vacuum. Next, a thin film of silver is 40 formed on the surface of member 26 by heating filament 19 to evaporate silver from the silver beads 21. This silver film is about 25% transparent.

45 The next step is to introduce oxygen into the 50

envelope 1 and oxidize the thin silver layer. The oxidization may be produced by the use of a high frequency discharge in the tube as described in Essig Patent 2,020,305. The resulting silver oxide layer 27 is about 80% to 90% transparent and is an insulator.

The envelope 1 is again pumped to a high vacuum and the silver oxide layer 27 is next sensitized in the usual manner. This consists 10 in admitting caesium or some other alkali metal from a side tube (not shown) and then baking the complete tube to cause the caesium to react with the silver oxide. This results in a layer 28 which probably is caesium oxide with a thin 15 layer of free caesium on the surface.

If sufficient caesium has been added, the film may be conducting and will show fair photoelectric sensitivity. However, the stability of such a film as regards conductivity is poor.

20 To overcome this defect, the next step is to evaporate from the beads 21 a very thin transparent layer 29 of silver upon the sensitized surface. The final step is to again bake the tube, this baking being similar to the previous 25 one which was used to cause a reaction between the caesium and the silver oxide. This results in a large increase in photoelectric sensitivity and, at the same time, the additional silver layer 29 adds the necessary conductivity 30 to the photoelectric surface.

It will be understood, of course, that the illustration in Fig. 3 is diagrammatic in that the various layers on the member 26 are too thin 35 to be shown in their true thickness. Also, it is likely that the several layers are intermixed to a certain extent not indicated on the drawing.

From the foregoing description it will be apparent that by oxidizing completely through the 40 first silver layer and allowing this oxide to react with caesium, we have the active photoelectric layer directly accessible to light passing through the member 26. At the same time we have a very sensitive surface which is conducting 45 cause of the outside silver layer.

I claim as my invention:

1. An electric discharge tube comprising an envelope having therein a transparent cathode supporting surface, a focusing electrode and an 50 anode located in the order named along the axis of the tube, said focusing electrode comprising two concentric rings having the space therebetween closed on the side facing said anode by a washer-like disc forming an annular recess 55 facing said cathode surface, and a filament mounted in said recess and having silver thereon which is located about said annular recess whereby silver may be evaporated upon said cathode supporting surface.

60 2. The invention according to claim 1 wherein the silver on said filament is in the form of

beads which are substantially uniformly spaced around said annular recess.

3. An electric discharge tube comprising an envelope having therein a transparent cathode supporting surface and a plurality of annular electrodes located along the axis of said tube, one of said electrodes comprising two concentric annular surfaces having the space therebetween closed on the side opposite said cathode supporting surface by a washer-like disc forming an annular recess facing said cathode surface, and a filament mounted in said recess and having a metal thereon which vaporizes at a substantially lower temperature than said filament whereby said metal may be evaporated upon said cathode surface.

4. An electric discharge tube comprising a transparent photoelectric cathode adapted to have a light image formed on one side thereof whereby a corresponding image of electrons is released from the opposite side thereof, said cathode comprising a transparent supporting surface, a transparent layer of silver oxide on and in contact with said surface, a transparent photoelectric sensitized surface on said silver oxide, a transparent layer of metal on said photoelectric surface which layer provides the necessary conductivity for said cathode to avoid distortion in the focusing of said electron image, and means for focusing said image of electrons in a plane removed from said cathode.

20 5. The invention according to claim 4 wherein said layer of metal is a layer of silver.

6. An electric discharge tube comprising a transparent photoelectric cathode adapted to have a light image formed on one side thereof whereby a corresponding image of electrons is released from the opposite side thereof, said cathode comprising a transparent supporting surface, a transparent layer of silver oxide on said surface, said layer being photo-sensitive on the surface farthest removed from said supporting surface, a transparent layer of silver on said photo-sensitive surface, and means for producing an electrostatic focusing field for focusing 40 said image of electrons in a plane removed from said cathode, said layer of silver being thick enough to give said cathode sufficiently good conductivity to prevent distortion of said focusing field near the cathode due to a potential 45 gradient along the cathode surface.

7. The invention according to claim 6 wherein said layer of silver oxide has been photo-sensitized by means of an alkali metal whereby there is a transparent alkali metal oxide surface on said silver oxide.

8. The invention according to claim 6 wherein said layer of silver oxide has been photo-sensitized by caesium whereby there is a transparent caesium oxide surface on said silver oxide.

60 LESLIE E. FLORY.